

# United States Patent Office

3,057,761

Patented Oct. 9, 1962

1

3,057,761

## COLORING OXIDE COATED ALUMINUM AND PRODUCT

Henry J. Wittrock, Opportunity, Wash., assignor to Kaiser Aluminum & Chemical Corporation, Oakland, Calif., a corporation of Delaware  
No Drawing. Filed May 9, 1960, Ser. No. 27,481  
22 Claims. (Cl. 148—6.1)

This invention relates to the production of colored coatings on aluminum and aluminum base alloys. More particularly, this invention relates to the coloring of oxide coatings on aluminum and aluminum base alloys characterized by stability in natural sunlight or ultra-violet light, and to the articles produced thereby.

For many purposes aluminum surfaces are protected by an oxide coating produced on the surface either by chemical treatment or by exposure as an anode in an electrolyte capable of yielding oxygen on electrolysis. The operation of forming such coatings electrolytically is commonly termed "anodizing" and the aluminum surface thus protected commonly termed "anodized." Such treatments generally provide colorless, grayish layers of oxide coating on aluminum. It has long been desired to color such oxide coated aluminum surfaces. In the past, such colored surfaces have been produced by first anodizing or chemically treating the aluminum metal base and thereafter, dyeing the oxide coating with organic dyes. Such processes possess certain inherent disadvantages with regard to color stability in natural sunlight or under ultra-violet light in that the colors tend to fade rapidly when exposed under such conditions.

This invention comprises immersing oxide coated aluminum metal in a warm aqueous solution of a salt of aurintricarboxylic acid selected from the group consisting of the sodium, potassium and ammonium salts, after which it is immersed in a warm aqueous solution of a salt having the general formula MX, where M is a metal selected from the group consisting of chromium, copper and cobalt, and X is an anion selected from the group consisting of sulfates, acetates, chlorides and nitrates. Next, the aluminum metal is immersed in a sulfuric acid solution and again immersed in a warm aqueous solution of a salt of aurintricarboxylic acid selected from the group consisting of the sodium, potassium and ammonium salts. If desired, the first immersion in the aqueous solution of the salt of aurintricarboxylic acid may be eliminated in some instances and a colored aluminum metal surface with good light stability may be produced. Further, good light stability and color may be achieved in some instances if the intermediate step of immersion in a warm aqueous salt solution having the general formula MX is eliminated or if the immersion in sulfuric acid is eliminated. However, immersion in either the salt solution having the general formula MX or the sulfuric acid is essential and for superior results with regard to light stability and color in general, it is preferred to include all the above recited steps. In some instances, further improvements with regard to light stability may be obtained by immersion of the metal in a pretreatment solution prior to the first immersion in the salt of aurintricarboxylic acid. For this pretreatment, it is preferred to employ an aqueous solution of ammonium bifluoride and nitric acid. Additional suitable pretreatment solutions include an aqueous 5% sulfuric acid solution and an aqueous 5% phosphoric acid solution.

Depending on the lustre or brightness of the colored aluminum metal desired, that is the degree of specular reflectance, the aluminum metal may be subjected to various treatments prior to anodizing. For example, where high lustre or brightness is desired, the base metal

2

may be subjected to conventional polishing or brightening treatments, e.g. mechanical, chemical or electrochemical. Where it is desired that the ultimate article have a matte or satin appearance, the base metal may be subjected to a suitable etching treatment. An example of a satisfactory procedure embodying the principles of this invention is set forth below, it being understood that the conventional water rinsing operations after the various steps are not recited.

- (1) Clean metal in an inhibited alkaline cleaner.
  - (2) (a) Where high lustre or brightness of the ultimate colored composite is desired, treat metal according to a suitable bright dip process.
  - (b) Where a matte appearance is desired in the ultimate composite, subject material to a caustic etch treatment in a solution of 5% sodium hydroxide plus 2% sodium fluoride maintained at a temperature of 160° F. for a 5-minute immersion period.
  - (3) Produce a porous oxide coating by oxidation of the surface layer of the aluminum by chemical or electrochemical means such as by chemical conversion or by anodizing. For example, anodize for 1 to 120 minutes in an electrolyte consisting essentially of an aqueous solution of from 5% to 30% sulfuric acid maintained at a temperature of from 30 to 100° F. The current density may range from about 5 to 30 a.s.f. and the voltages may range from about 0 to 30 volts. As used herein, the term "a.s.f." is an abbreviation or contraction of the expression "amperes per square foot."
  - (4) Immerse for from 5 seconds to 2 minutes in an aqueous solution of from 2 to 100 grams per liter of a salt of aurintricarboxylic acid selected from the group consisting of the sodium, potassium and ammonium salts having a pH of from 3 to 8, and a temperature of from 120 to 185° F.
  - (5) Immerse for from 2 to 7 minutes in an aqueous solution of one of the following salts: chromium sulfate, chromium acetate, chromium chloride, chromium nitrate, copper sulfate, copper acetate, copper chloride, copper nitrate, cobalt sulfate, cobalt acetate, cobalt chloride and cobalt nitrate. The concentration should range from 1 gram of salt per liter of water to saturation and the solution should have a pH of from 1 to 4 and a temperature of from 120-160° F.
  - (6) Rinse for from 15 seconds to 5 minutes in an aqueous solution of sulfuric acid having a concentration of from .05 to .5% by weight H<sub>2</sub>SO<sub>4</sub>, a pH of from 1 to 3, and a temperature ranging from room temperature (70° F.) to 150° F.
  - (7) Immerse for from 2 to 10 minutes in an aqueous solution of from 2 to 100 grams per liter of a salt of aurintricarboxylic acid selected from the group consisting of the sodium, potassium and ammonium salts having a pH of from 3 to 8 and a temperature of from 120 to 185° F.
  - (8) The oxide coatings may be sealed by a conventional sealing treatment, e.g., immersion in hot water maintained at a temperature of from 180 to 200° F. and a pH of from 5-6 for a period of from 10 to 30 minutes.
  - The aluminum metal should then be rinsed in distilled water and dried.
- In order to establish the superior light fastness of the colored anodic oxide coatings produced in accordance with this invention and the composite article coated therewith over those produced by conventional prior art methods, tests described hereinbelow have been conducted.
- In these tests, samples were fabricated from sheets of aluminum alloys 5357 and 1100 cut into 1" by 3" rectangles providing a total surface area of about 6 square inches per sample. The 5357 alloy samples had the following composition in percent by weight: silicon 0.08, iron 0.11, copper 0.01, manganese 0.28, magnesium 1.00,

zinc 0.01, titanium 0.02, balance aluminum. The 1100 alloy samples were commercially pure aluminum containing a minimum of 99% aluminum.

In these tests the samples were treated as indicated below, it being understood that the conventional cold water rinsing operations after the various steps are not recited:

(1) All samples were cleaned to a water-break free surface in a mild inhibited alkaline cleaner of the type containing a mixture of carbonates, phosphates and silicates maintained at 160° F. Samples 1-14 were etched for five minutes in an aqueous solution of 5% sodium hydroxide and 2% sodium fluoride at a temperature of 160° F. Samples 15 and 16 were bright dipped in a solution containing 80.3% by weight  $H_3PO_4$ , 3.8% by weight  $HNO_3$ , balance water maintained at a temperature of about 200° F. for a period of about 2 minutes.

(2) Samples 1-14 were rinsed for 15 seconds in 50% by volume nitric acid at room temperature.

(3) All samples were anodized in a 50 gallon rectangular tank equipped with stirring devices and lead cathodes for 30 minutes with direct current in an aqueous sulfuric acid electrolyte containing 15% by weight  $H_2SO_4$  at a temperature of 70° F. The current density was maintained at 12 a.s.f. In general, the voltages necessary to maintain a given current density vary with the cell and the anodizing conditions and the required voltage varies as the anodizing progresses. In anodizing the samples employed in these tests, the voltages required to maintain a constant current density of 12 a.s.f. ranged from about 2 to 17 volts.

(4) Sample 6 was immersed for ten seconds in a room temperature (70° F.) aqueous pretreatment solution containing 25 g./l.  $NH_4HF_2$ , 15 ml./l.  $HNO_3$  (70%), balance water. The solution was contained in a 1 liter beaker.

(5) Samples of 1-6 and 15 were immersed in an aqueous solution of the salt of aurintricarboxylic acid indicated in the table having a concentration of 10 grams of salt per liter of water for a period of one minute. In the table aurintricarboxylic acid is indicated by A.T.C.

ous solution of sulfuric acid contained in a 1 liter beaker. Samples 1-3 and 6 were immersed 15 seconds in a .05% by weight aqueous sulfuric acid solution having a pH of 3 at room temperature. Sample number 5 was immersed for five minutes in a .5% by weight aqueous solution of sulfuric acid having a pH of 2 and a temperature of 150° F. Step number 7 was not employed with sample number 4.

(8) All samples were immersed for 5 minutes in an aqueous solution of a salt of aurintricarboxylic acid as indicated in the table having a concentration of 10 grams of salt per liter of water. This solution was maintained at a pH of 5 and at a temperature of 150° F. and was contained in a 1 liter beaker.

(9) All samples were sealed by immersion in boiling distilled water for 10 minutes, rinsed in distilled water and dried.

All the samples treated as above described were characterized by a red color having a pleasing appearance.

20 The superiority of the method of this invention is clearly demonstrated by a comparison of the dye life of samples 1-6 and 15 employing the method of this invention with samples 7-14 and 16 employing a single dyeing treatment without either of the intermediate steps 25 6 and 7. Dye life was determined by measuring diffuse reflectance whereby a gain in diffuse reflectance indicates fading. A 25% gain in diffuse reflectance is approximately the maximum permissible for commercial acceptability. Each sample was subjected to ultra-violet 30 light in a testing box and the number of hours in such test box required for a 25% gain in diffuse reflectance determined. The number of hours for each sample is indicated in the table. For good light stability it is desirable to have a dye life greater than 300 hours. It 35 will be seen from the table that none of the samples 7-14 and 16 employing the prior art method has a dye life as great as 300 hours and many of these samples had a very short dye life. However, samples 1-6 and 15 all had a dye life greater than 300 hours thereby demonstrating the superiority of the method of this invention and the articles produced thereby.

Table

| Sample No. | Alloy | Step 5<br>Salt of<br>A.T.C. | Step 6                                                                |       |     | Step 8<br>Salt of<br>A.T.C. | Dye<br>Life |
|------------|-------|-----------------------------|-----------------------------------------------------------------------|-------|-----|-----------------------------|-------------|
|            |       |                             | Salt                                                                  | g./l. | pH  |                             |             |
| 1          | 5357  | NH <sub>4</sub>             |                                                                       |       |     |                             |             |
| 2          | 5357  | NH <sub>4</sub>             | Cr <sub>2</sub> (SO <sub>4</sub> ) <sub>3</sub>                       | 7.3   | 1.5 | NH <sub>4</sub>             | 400         |
| 3          | 5357  | NH <sub>4</sub>             | CuSO <sub>4</sub>                                                     | 10    | 4.5 | NH <sub>4</sub>             | 510         |
| 4          | 5357  | NH <sub>4</sub>             | CuCl <sub>2</sub>                                                     | 10    | 4.1 | NH <sub>4</sub>             | 410         |
| 5          | 5357  | NH <sub>4</sub>             | {CoSO <sub>4</sub> 10 g./l. + H <sub>2</sub> SO <sub>4</sub> 2 ml./l. | 1.9   |     | NH <sub>4</sub>             | 370         |
| 6          | 5357  | NH <sub>4</sub>             |                                                                       |       |     | NH <sub>4</sub>             | 500         |
| 7          | 5357  | NH <sub>4</sub>             | Cr <sub>2</sub> (SO <sub>4</sub> ) <sub>3</sub>                       | 7.3   | 1.5 | NH <sub>4</sub>             | 740         |
| 8          | 5357  |                             |                                                                       |       |     | NH <sub>4</sub>             | 160         |
| 9          | 5357  |                             |                                                                       |       |     | NH <sub>4</sub>             | 190         |
| 10         | 5357  |                             |                                                                       |       |     | NH <sub>4</sub>             | 190         |
| 11         | 5357  |                             |                                                                       |       |     | N <sub>3</sub>              | 150         |
| 12         | 5357  |                             |                                                                       |       |     | N <sub>3</sub>              | 160         |
| 13         | 5357  |                             |                                                                       |       |     | NH <sub>4</sub>             | 80          |
| 14         | 5357  |                             |                                                                       |       |     | NH <sub>4</sub>             | 50          |
| 15         | 1100  | Na                          | Cr(C <sub>2</sub> H <sub>3</sub> O <sub>2</sub> ) <sub>3</sub>        | 5     | 1.5 | NH <sub>4</sub>             | 100         |
| 16         | 1100  |                             |                                                                       |       |     | Na                          | 410         |
|            |       |                             |                                                                       |       |     | K                           | 70          |

The solution was contained in a 1 liter beaker. The pH of the solution was 5 and the temperature was 150° F.

(6) Samples 1-4, 6 and 15 were immersed for five minutes in an aqueous solution of a salt having the general formula MX, where M is a metal selected from the group consisting of chromium, copper and cobalt, and where X is an anion selected from the group consisting of sulfates, nitrates, acetates and chlorides. This solution was contained in a 1 liter beaker. The salt employed, the concentration in grams of salt per liter of water and pH are indicated in the table. The solution was maintained at a temperature of 150° F. Step number 6 was not employed with sample No. 5.

(7) Samples 1-3, 5 and 6 were immersed in an aque-

ous solution of sulfuric acid contained in a 1 liter beaker. Samples 1-3 and 6 were immersed 15 seconds in a .05% by weight aqueous sulfuric acid solution having a pH of 3 at room temperature. Sample number 5 was immersed for five minutes in a .5% by weight aqueous solution of sulfuric acid having a pH of 2 and a temperature of 150° F. Step number 7 was not employed with sample number 4.

(8) All samples were immersed for 5 minutes in an aqueous solution of a salt of aurintricarboxylic acid as indicated in the table having a concentration of 10 grams of salt per liter of water. This solution was maintained at a pH of 5 and at a temperature of 150° F. and was contained in a 1 liter beaker.

(9) All samples were sealed by immersion in boiling distilled water for 10 minutes, rinsed in distilled water and dried.

All the samples treated as above described were characterized by a red color having a pleasing appearance.

20 The superiority of the method of this invention is clearly demonstrated by a comparison of the dye life of samples 1-6 and 15 employing the method of this invention with samples 7-14 and 16 employing a single dyeing treatment without either of the intermediate steps 25 6 and 7. Dye life was determined by measuring diffuse reflectance whereby a gain in diffuse reflectance indicates fading. A 25% gain in diffuse reflectance is approximately the maximum permissible for commercial acceptability. Each sample was subjected to ultra-violet 30 light in a testing box and the number of hours in such test box required for a 25% gain in diffuse reflectance determined. The number of hours for each sample is indicated in the table. For good light stability it is desirable to have a dye life greater than 300 hours. It 35 will be seen from the table that none of the samples 7-14 and 16 employing the prior art method has a dye life as great as 300 hours and many of these samples had a very short dye life. However, samples 1-6 and 15 all had a dye life greater than 300 hours thereby demonstrating the superiority of the method of this invention and the articles produced thereby.

What is claimed is:

1. In the art of coloring oxide coatings on aluminum metal, the improvement comprising the steps of immersing the oxide coated aluminum metal in an aqueous solution of a salt of aurintricarboxylic acid selected from the group consisting of the sodium, potassium and ammonium salts, immersing the so-treated aluminum metal in an aqueous

solution of a salt having the general formula  $MX$ , wherein  $M$  is a metal selected from the group consisting of chromium, copper and cobalt, and  $X$  is an anion selected from the group consisting of sulfates, acetates, chlorides and nitrates, followed by immersion in an aqueous solution of sulfuric acid, and immersing the aluminum metal for a second time in an aqueous solution of a salt of aurintricarboxylic acid selected from the group consisting of the sodium, potassium and ammonium salts.

2. The method of claim 1 wherein the oxide coated aluminum metal is immersed in a pretreatment solution prior to the first immersion in the salt of aurintricarboxylic acid. 10

3. The method of claim 2 wherein said pretreatment solution is an aqueous solution of ammonium bifluoride and nitric acid.

4. In the art of coloring oxide coatings on aluminum metal, the improvement comprising the steps of immersing the oxide coated aluminum metal in an aqueous solution of a salt of aurintricarboxylic acid selected from the group consisting of the sodium, potassium and ammonium salts, immersing the so-treated aluminum metal in an aqueous solution of sulfuric acid followed by a second immersion of the aluminum metal in an aqueous solution of a salt of aurintricarboxylic acid selected from the group consisting of the sodium, potassium and ammonium salts.

5. In the art of coloring oxide coatings on aluminum metal, the improvement comprising the steps of immersing the oxide coated aluminum metal in an aqueous solution of a salt having the general formula  $MX$ , wherein  $M$  is a metal selected from the group consisting of chromium, copper and cobalt, and  $X$  is an anion selected from the group consisting of sulfates, acetates, chlorides and nitrates, immersing the so-treated aluminum metal in an aqueous solution of sulfuric acid and finally immersing the aluminum metal in an aqueous solution of a salt of aurintricarboxylic acid selected from the group consisting of the sodium, potassium and ammonium salts.

6. In the art of coloring oxide coatings on aluminum metal, the improvement comprising the steps of immersing the oxide coated aluminum metal in an aqueous solution of a salt of aurintricarboxylic acid selected from the group consisting of the sodium, potassium and ammonium salts, immersing the so-treated aluminum metal in an aqueous solution of a salt having the general formula MX, wherein M is a metal selected from the group consisting of chromium, copper and cobalt, and X is an anion selected from the group consisting of sulfates, acetates, chlorides and nitrates, and finally immersing the aluminum metal for a second time in an aqueous solution of a salt of aurintricarboxylic acid selected from the group consisting of the sodium, potassium and ammonium salts.

sodium, potassium and ammonium salts having a pH of from 3 to 8 and a temperature of from 120 to 185° F., immersing the so-treated aluminum metal for from 2 to 7 minutes in an aqueous solution of a salt having the general formula  $MX$ , wherein M is a metal selected from the group consisting of chromium, copper and cobalt and X is an anion selected from the group consisting of sulfates, acetates, chlorides and nitrates, said salt being in a concentration ranging from 1 gram of salt per liter of water to saturation having a pH of from 1 to 4 and a temperature from 120 to 160° F., followed by immersion of the aluminum metal for from 15 seconds to 5 minutes in an aqueous solution of from .05 to .5% by weight sulfuric acid having a pH of from 1 to 3 and a temperature of from 70 to 150° F., and immersing the aluminum metal for from 2 to 10 minutes in an aqueous solution of from 2 to 100 grams per liter of a salt of aurintricarboxylic acid selected from the group

consisting of the sodium, potassium and ammonium salts having a pH of from 3 to 8 and a temperature from 120 to 185° F.

8. The method of claim 7 wherein the metal M in the general formula MX is chromium.

9. The method of claim 7 wherein the metal M in the general formula MX is copper.

10. The method of claim 7 wherein the metal M in the general formula MX is cobalt.

11. The method of claim 7 wherein the anion X in the general formula MX is a sulfate.

12. The method of claim 7 wherein the anion X in the general formula MX is an acetate.

13. The method of claim 7 wherein the anion X in the general formula MX is a chloride.

14. The method of claim 7 wherein the anion X in the general formula MX is a nitrate.

15. The method of claim 7 wherein the salt of aurintricarboxylic acid is the ammonium salt.

16. The method of claim 7 wherein the salt of aurintricarboxylic acid is the sodium salt.

17. The method of claim 7 wherein the salt of aurintricarboxylic acid is the potassium salt.

18. In the art of coloring anodic oxide coatings on

16. In the art of ~~coating~~  
aluminum metal, the improvement comprising the steps  
of immersing the oxide coated aluminum metal for  
from 2 to 7 minutes in an aqueous solution of a salt  
having the general formula  $MX$ , wherein M is a metal  
selected from the group consisting of chromium, copper  
and cobalt and X is an anion selected from the group  
consisting of sulfates, acetates, chlorides and nitrates, the  
concentration of said salt ranging from 1 gram of salt  
per liter of water to saturation, said solution having a  
pH of from 1 to 4 and a temperature from 120 to  
160° F., followed by immersion for from 15 seconds to  
5 minutes in an aqueous solution of from .05 to .5%  
by weight sulfuric acid having a pH of from 1 to 3 and  
a temperature of from 70 to 150° F., and immersing  
the aluminum metal for from 2 to 10 minutes in an  
aqueous solution of from 2 to 100 grams per liter of a  
salt of aurintricarboxylic acid selected from the group  
consisting of the sodium, potassium, and ammonium salts  
maintained at a pH of from 3 to 8 and a temperature  
from 120 to 185° F.

5 19. In the art of coloring anodic oxide coatings on aluminum metal, the improvement comprising the steps of immersing the oxide coated aluminum metal for from 5 seconds to 2 minutes in an aqueous solution of from 2 to 100 grams per liter of a salt of aurintricarboxylic

acid selected from the group consisting of the sodium, potassium and ammonium salts having a pH of from 3 to 8 and a temperature of from 120 to 185° F., followed by immersion of the aluminum metal for from 15 sec-

by immersion of the aluminum metal for from 1 to 10 seconds to 5 minutes in an aqueous solution of from .05 to .5% by weight sulfuric acid having a pH of from 1 to 3 and a temperature of from 70 to 150° F., and immersing the aluminum metal for from 2 to 10 minutes in an aqueous solution of from 2 to 100 grams per liter

in an aqueous solution of a salt of aurintricarboxylic acid selected from the group consisting of the sodium, potassium and ammonium salts having a pH of from 3 to 8 and a temperature of from 120 to 185° F.

20. In the art of coloring anodic oxide coatings on aluminum metal, the improvement comprising the steps

aluminum metal, the improvement comprising the steps  
65 of immersing the oxide coated aluminum metal for from  
5 seconds to 2 minutes in an aqueous solution of from  
2 to 100 grams per liter of a salt of aurintricarboxylic  
acid selected from the group consisting of the sodium,  
potassium and ammonium salts having a pH of from 3

potassium and ammonium salts having a pH of 7 to 8 and a temperature of from 120 to 185° F., immersing the so-treated aluminum metal for from 2 to 7 minutes in an aqueous solution of a salt having the general formula MX, wherein M is a metal selected from the group consisting of chromium, copper and cobalt and X is an anion selected from the group con-

sisting of sulfates, acetates, chlorides and nitrates, said salt being in a concentration ranging from 1 gram of salt per liter of water to saturation having a pH of from 1 to 4 and a temperature from 120 to 160° F., and immersing the aluminum metal for from 2 to 10 minutes in an aqueous solution of from 2 to 100 grams per liter of a salt of aurintricarboxylic acid selected from the group consisting of the sodium, potassium and ammonium salts having a pH of from 3 to 8 and a temperature from 120 to 185° F.

21. In the art of coloring anodic oxide coatings on aluminum metal, the improvement comprising the steps of immersing the oxide coated aluminum metal for about 10 seconds in an aqueous solution containing about 25 grams per liter of ammonium bifluoride, 15 milliliters per liter of 70% nitric acid, balance water, followed by immersion of said aluminum metal for from 5 seconds to 2 minutes in an aqueous solution of from 2 to 100 grams per liter of a salt of aurintricarboxylic acid selected from the group consisting of the sodium, potassium and ammonium salts having a pH of from 3 to 8 and a temperature of from 120 to 185° F., immersing the so-treated aluminum metal from from 2 to 7 minutes in an aqueous solution of a salt having the general formula MX, wherein M is a metal selected from the group consisting of chromium, copper and cobalt and X is an anion selected from the group consisting of sulfates, acetates, chlorides and nitrates, said salt being in a concentration ranging from 1 gram of salt per liter of water to saturation, having a pH of from 1 to 4 and a temperature from 120 to 160° F., followed by immersion of the aluminum metal for 15 seconds to 5 minutes in an aqueous solution of from .05 to .5% by weight sulfuric acid having a pH of from 1 to 3 and a temperature of from 70 to 150° F., and immersing the aluminum metal from from 2 to 10 minutes in an aqueous solution of from 2 to 100 grams per

8  
liter of a salt of aurintricarboxylic acid selected from the group consisting of the sodium, potassium, and ammonium salts having a pH of from 3 to 8 and a temperature from 120 to 185° F.

- 5 22. A composite article comprising a base portion of aluminum metal and a red colored anodic oxide coating adhering thereto characterized by a pleasing appearance and superior light fastness produced by immersing an oxide coated aluminum article in an aqueous solution of 10 a salt of aurintricarboxylic acid, selected from the group consisting of the sodium, potassium and ammonium salts followed by immersing the so-treated aluminum metal in an aqueous solution of a salt having the general formula MX wherein M is a metal selected from the group consisting of 15 chromium, copper and cobalt, and X is an anion selected from the group consisting of sulfates, acetates, chlorides and nitrates, followed by immersion in an aqueous solution of sulfuric acid, and finally immersing the article for a second time in an aqueous solution of 20 a salt of aurintricarboxylic acid selected from the group consisting of the sodium, potassium and ammonium salts.

References Cited in the file of this patent

25

UNITED STATES PATENTS

- 1,946,148 Tosterud ----- Feb. 3, 1934  
2,071,156 Baer ----- Feb. 16, 1937  
2,538,317 Mason et al. ----- Jan. 16, 1951  
2,538,831 Cutter ----- Jan. 23, 1951

30

FOREIGN PATENTS

- 387,806 Great Britain ----- Feb. 16, 1933

35

OTHER REFERENCES

- Lederer et al.: "Chromatography," second edition, page 232.

UNITED STATES PATENT OFFICE  
CERTIFICATE OF CORRECTION

Patent No. 3,057,761

October 9, 1962

Henry J. Wittrock

It is hereby certified that error appears in the above numbered patent requiring correction and that the said Letters Patent should read as corrected below.

Column 2, line 60, for "rised" read -- rinsed --; column 3, line 37, for "immsersed" read -- immersed --; column 6, line 23, for "poassium" read -- potassium --; column 7, line 35, for "metal from from" read -- metal for from --; column 8, line 8, for "fastless" read -- fastness --.

Signed and sealed this 21st day of May 1963.

(SEAL)

Attest:

ERNEST W. SWIDER  
Attesting Officer

DAVID L. LADD  
Commissioner of Patents